

# United States Patent [19]

Najjar et al.

[11] Patent Number: 4,946,476

[45] Date of Patent: Aug. 7, 1990

[54] PARTIAL OXIDATION OF BITUMINOUS COAL

[75] Inventors: **Mitri S. Najjar**, Wappingers Falls; **Walter C. Gates, Jr.**, Carmel, both of N.Y.

[73] Assignee: **Texaco Inc.**, White Plains, N.Y.

[21] Appl. No.: 397,945

[22] Filed: Aug. 24, 1989

[51] Int. Cl.<sup>5</sup> ..... C10J 3/46

[52] U.S. Cl. ..... 48/197 R; 48/206; 48/215; 252/373

[58] Field of Search ..... 48/197 R, 202, 206, 48/215, DIG. 7; 252/373

[56] References Cited

U.S. PATENT DOCUMENTS

|           |         |                  |          |
|-----------|---------|------------------|----------|
| 2,818,326 | 12/1957 | Eastman et al.   | 48/196   |
| 2,931,715 | 4/1960  | Eastman          | 48/63    |
| 3,544,291 | 12/1970 | Schlinger et al. | 48/206   |
| 3,607,157 | 9/1971  | Schlinger et al. | 48/206   |
| 3,620,900 | 11/1971 | Schlinger et al. | 48/216   |
| 3,847,564 | 11/1974 | Marion et al.    | 48/95    |
| 3,951,617 | 4/1976  | Crouch           | 48/2 F   |
| 3,998,609 | 12/1976 | Crouch et al.    | 48/197   |
| 4,060,397 | 11/1977 | Buiter et al.    | 48/197 R |
| 4,074,981 | 2/1978  | Slater           | 48/197 R |
| 4,081,253 | 3/1978  | Marion           | 48/197   |
| 4,099,383 | 7/1978  | Paull et al.     | 48/197 R |
| 4,218,423 | 8/1980  | Robin et al.     | 422/207  |
| 4,255,278 | 3/1981  | Roberts et al.   | 48/197 R |
| 4,289,502 | 9/1981  | Muenger et al.   | 48/62    |
| 4,364,744 | 12/1982 | Crouch et al.    | 48/86    |
| 4,377,132 | 3/1988  | Koog et al.      | 122/7    |
| 4,392,981 | 7/1983  | Corbeels et al.  | 48/206   |

|           |         |               |         |
|-----------|---------|---------------|---------|
| 4,525,175 | 6/1985  | Stellaccio    | 48/86   |
| 4,547,203 | 10/1985 | Jaluke        | 48/206  |
| 4,657,698 | 4/1987  | Najjar et al. | 252/373 |
| 4,668,428 | 5/1987  | Najjar        | 252/373 |
| 4,668,429 | 5/1987  | Najjar        | 252/373 |
| 4,676,805 | 6/1987  | Richter       | 48/206  |
| 4,732,700 | 3/1988  | Najjar et al. | 252/373 |
| 4,826,627 | 5/1989  | Najjar        | 252/373 |

Primary Examiner—Peter Kratz

Attorney, Agent, or Firm—Robert A. Kulason; James J. O'Loughlin; Albert Brent

[57] ABSTRACT

Synthesis gas, reducing gas, or fuel gas is produced by the partial oxidation of bituminous coal at an autogenous temperature in the range of about 2000° F. to 2700° F. and at a pressure in the range of about 17 to 100 atmospheres to produce a raw effluent gas stream containing entrained molten slag and carbon-rich particulate material. After cooling, course slag and carbon-rich particulate material are separated. A fuel mixture comprising about 20 to 100 wt. % of said carbon-rich particulate material and the remainder comprising a supplemental fuel is reacted by partial oxidation at an autogenous temperature of about 2000° F. to 2700° F. and at a reduced pressure e.g. in the range of about 1 to 16 atmospheres and at least 16 atmospheres below the pressure in the partial oxidation reaction used to produce said carbon-rich particulate material. By reducing the pressure less carbon-rich particulate material is produced in the second partial oxidation reaction at a significant cost savings and improved process efficiency.

13 Claims, No Drawings

## PARTIAL OXIDATION OF BITUMINOUS COAL

## FIELD OF THE INVENTION

This invention relates to a partial oxidation process for producing synthesis gas, reducing gas, or fuel gas starting with bituminous coal.

## DESCRIPTION OF THE PRIOR ART

The partial oxidation of liquid hydrocarbon fuels e.g. petroleum and solid carbonaceous fuel e.g. coal to produce synthesis gas, reducing gas, and fuel gas is a well known process. These man-made gas mixtures all contain hydrogen, carbon monoxide and at least one gas from the group consisting of  $H_2O$ ,  $CO_2$ ,  $N_2$ ,  $H_2S$ ,  $COS$ ,  $CH_4$ , and mixtures thereof. Prior to gas quenching or scrubbing the raw gas stream also contains entrained molten slag containing carbonaceous materials. Synthesis gas contains a  $H_2/CO$  mole ratio which may be specified over a wide range. It is used as the gaseous feedstock for the catalytic synthesis of organic chemicals e.g. alcohol. Reducing gas is a gaseous mixture substantially comprising  $H_2+CO$  and is used in metallurgical processes to effect reduction. Fuel gas is rich in  $H_2$ ,  $CO$  and contains  $CH_4$ . It is used for heating. The hot raw gas stream from the partial oxidation gas generator may also contain entrained molten slag, fly-ash, and unreacted carbon-rich material. The composition of these gases depends upon actual feedstreams and the reaction conditions.

Recovering particulate carbon from raw synthesis gas and recycling the carbon in admixture with coal back to the gas generator as a portion of the feed is shown and described in coassigned U.S. Pat. No. 3,544,291, which is incorporated herein by reference. The carbon soot recovered from two gas generators is mixed with a heavy liquid hydrocarbon fuel and recycled to one of the gas generators in coassigned U.S. Pat. No. 4,411,670. However, the prior art references do not teach or suggest applicants' improved process by which the hot raw product gas streams from the partial oxidation of bituminous coal is cooled and separated into synthesis gas, course slag and carbon-rich particulate material. The carbon-rich particulate material, with or without being mixed with a supplemental fuel, is then reacted by partial oxidation at a substantially reduced pressure. Synthesis gas is thereby produced by the subject process containing substantially less carbon-rich particulate material at a significant cost savings and improved process efficiency.

## SUMMARY OF THE INVENTION

This invention relates to an improved partial oxidation process for producing synthesis gas, reducing gas or fuel gas from bituminous coal comprising the steps of:

(1) reacting said bituminous coal by partial oxidation with a free-oxygen containing gas and a temperature moderator in a free-flow vertical refractory-lined gas generator at an autogenous temperature in the range of about 2000° F. to 2700° F., a pressure in the range of about 17 to 100 atmospheres, an O/C atomic ratio in the range of about 0.7 to 1.6, and a weight ratio of  $H_2O$  to bituminous coal in the range of about 0.10 to 5.0, to produce a raw gas stream comprising synthesis gas, reducing gas, or fuel gas with entrained molten slag and carbon-rich particulate material;

(2) cooling said raw gas stream from (1) and separating therefrom coarse slag and carbon-rich particulate material;

(3) reacting a fuel mixture comprising from about 5 to 100 wt. % of said carbon-rich particulate material and any remainder comprising a supplemental fuel selected from the group consisting of liquid hydrocarbonaceous fuel, coal, petroleum coke, and mixtures thereof by partial oxidation with a free-oxygen containing gas and a temperature moderator in a free-flow vertical refractory-lined gas generator at an autogenous temperature in the range of about 2000° F. to 2700° F., a pressure in the range of about 1 to 16 atmospheres and at least 16 atmospheres below the pressure in the 10 gas generator in (1), an O/C atomic ratio in the range of about 0.6 to 1.3, and a weight ratio of  $H_2O$  to fuel mixture in the range of about 0.1 to 5.0, to produce a raw product gas stream comprising synthesis gas, reducing gas, or fuel gas with entrained molten slag and containing 15 less carbon-rich particulate material than that produced when said fuel mixture is reacted by partial oxidation at substantially the same operating conditions as those in the gas generator in (3) except for a higher pressure which is in the same range as that in the gas generator in (1); and

(4) cooling said raw gas stream from (3).

The partial oxidation reactions in (1) and (3) may take place in the same or different gas generators.

## DESCRIPTION OF THE INVENTION

Synthesis gas, reducing gas and fuel gas comprising mixtures of  $H_2$ ,  $CO$  and various amounts of other gases may be made by the partial oxidation process, such as described in coassigned U.S. Pat. Nos. 3,544,291, 3,607,157, 3,998,609 and 4,289,502, which are incorporated herein by reference. Advantageously, the partial oxidation process may use as feedstock comparatively low-cost readily available ash-containing solid carbonaceous fuels. For example, the following ash-containing solid carbonaceous fuels have been previously used: coal i.e. anthracite, bituminous, subbituminous, or lignite; coke from coal; petroleum coke; oil shale; tar sands; asphalt; pitch; and mixtures thereof. However, only bituminous coal is used as the starting solid fuel feedstock in the subject process.

It was generally believed that the amount of carbon conversion for any of the solid fuels increased as the gasification temperature and pressure are increased. For example, the steam and  $CO_2$  reactions with carbon to produce  $CO$  and  $H_2$  increase with pressure and temperature. However, it was unexpectedly found that by the subject process using bituminous coal, carbon conversion is increased with decreasing pressure. Advantageously, it is more economical to operate a gas generator at a lower pressure. Further, a greater amount of product gas is produced containing substantially less carbon-rich particulate material.

The term bituminous coal, as used herein, refers to Class II Bituminous Coal Groups 1 to 5 ASTM D 388-66.

In the subject partial oxidation process, ground solid bituminous coal may be introduced into the gas generator either alone or in the presence of a substantially thermally vaporizable hydrocarbon and/or water, or entrained in a temperature moderator such as steam,  $CO_2$ ,  $N_2$  or recycle synthesis gas. The particle size of the bituminous coal supplied to the gas generator is such that 100% passes through an ASTM E11-70 Sieve Des-

ignition Standard (SDS) 1.40 mm Alternative No. 14, such as about 425  $\mu$ m Alternative No. 40.

An annular-type burner is used to introduce the bituminous coal feed into the gasifier. Suitable annular-type burners are shown and described in coassigned U.S. Pat. Nos. 3,847,564; 4,364,744; and 4,525,175, which are incorporated herein by reference. The burner is located in the top of the gas generator along the central vertical axis. A typical down-flowing free-flow unobstructed vertical refractory lined partial oxidation synthesis gas generator is shown in coassigned U.S. Pat. No. 2,818,326, which is incorporated herein by reference.

The term free-oxygen containing gas, as used herein is intended to include air, oxygen-enriched air, i.e. greater than 21 mole % oxygen, and substantially pure oxygen i.e. greater than 95 mole % oxygen (the remainder comprising  $N_2$  and rare gases). Free oxygen containing gas may be introduced into the burner at a temperature in the range of about ambient to 1000° F.

The use of a temperature moderator to moderate the temperature in the reaction zone of the gas generator depends in general on the carbon to hydrogen ratio of the feedstock and the oxygen content of the oxidant stream. Suitable temperature moderators include steam, water,  $CO_2$ -rich gas, liquid  $CO_2$ , recycle synthesis gas, a portion of the cooled clean exhaust gas from a gas turbine employed downstream in the process, by-product nitrogen from the air separation unit used to produce substantially pure oxygen, and mixtures of the aforesaid temperature moderators. Water serves as the carrier and the temperature moderator with bituminous coal slurries. However, steam may be the temperature moderator with slurries of liquid hydrocarbon fuels and solid carbonaceous fuel. The temperature moderator may be introduced into the gas generator in admixture with either the solid carbonaceous fuel feed, the free-oxygen containing gas stream, or both. Alternatively, the temperature moderator may be introduced into the reaction zone of the gas generator by way of a separate conduit in the fuel burner. When  $H_2O$  is introduced into the gas generator either as a temperature moderator, a slurring medium, or both, the weight ratio of  $H_2O$  to fuel is in the range of about 0.1 to 5.0 and preferably in the range of about 0.2 to 1.0.

The relative proportions of solid carbonaceous fuel, liquid hydrocarbon fuel if any, water or other temperature moderator, and oxygen in the feed streams to gas generator, are carefully regulated to convert a substantial portion e.g. 75 to 95 wt. %, such as 80 to 90 wt. % of the carbon in the fuel feed to the partial oxidation gas generator to carbon oxides e.g.  $CO$  and  $CO_2$ ; and, to maintain an autogenous reaction zone temperature in the range of about 2000° F. to 2700° F. and above the ash-fusion temperature of the slag formed in the reaction zone. Advantageously, with bituminous coal feeds, the ash in the solid fuel forms molten slag at such reaction temperatures. Molten slag is much easier to separate from the hot effluent gas than fly ash. In the first partial oxidation reaction, the pressure in the reaction zone is in the range of about 17 to 100 atmospheres, and the atomic ratio of free-oxygen in the oxidant to carbon in the fuel feedstock (O/C atom/atom) is in the range of about 0.7 to 1.6. The time in the reaction zone of the partial oxidation gas generator in seconds is in the range of about 0.5 to 10, such as normally about 1.0 to 5. Reaction takes place in a reducing atmosphere.

The effluent gas stream leaving the partial oxidation gas generator has the following composition in mole %

:  $H_2$  8.0 to 60.0,  $CO$  8.0 to 70.0,  $CO_2$  1.0 to 50.0,  $H_2O$  2.0 to 50.0,  $CH_4$  0.0 to 2.0,  $H_2S$  plus  $COS$  0.10 to 2.0,  $N_2$  0.0 to 80.0, and  $A$  0.0 to 2.0. Trace amounts of the following gaseous impurities may be also present in the effluent gas stream in parts per million (ppm):  $HCN$  0 to 100; such as about 2 to 20;  $HCl$  0 to about 20,000, such as about 200 to 2,000; and  $NH_3$  0 to about 10,000, such as about 100 to 1000. Entrained in the effluent gas stream is about 1.0 to 10 wt. %, such as 2 to 4 wt. %, of porous carbon-rich particulate material (basis weight of carbon in the feed to the gas generator). Molten slag resulting from the fusion of the ash content in the coal is also entrained in the gas stream leaving the generator. Molten slag is the fused mineral matter of the bituminous coal feed. The content of mineral matter in bituminous coal is about 5 to 20 wt. %.

At least a portion e.g. about 20 to 100 volume % of the effluent gas stream leaving the reaction zone of partial oxidation gas generator is passed through the unobstructed central axial passage at the bottom of the reaction zone.

The hot raw effluent gas stream exits from the partial oxidation gas generator and may be cooled to a temperature in the range of about 60° to 950° F., such as less than about 350° F. For example, the hot gas stream may be first partially cooled by direct contact with water contained in a quench tank, such as shown in coassigned U.S. Pat. No. 4,218,423, which is incorporated herein by reference. Molten slag is solidified by the quench water and most of the coarse slag particles and carbon-rich particulate material are transferred to the water in the quench tank. The coarse slag particles comprise about 99 wt. % of inorganic materials and less than about 1 wt. % of unconverted carbon. The coarse slag material has a particle size of 40 mesh or more. The carbon-rich particulate matter comprises about 10 to 80 wt. % carbon, such as about 51.2 wt. %, about 20 to 90 wt. % ash, such as about 47.1 wt. %, and about 0 to 15 wt. % of  $H_2O$ , such as about 1.7 wt. %. The carbon-rich material has a particle size of less than about 40 mesh.

The partially cooled gas stream may be then passed through a water scrubbing operation to remove any remaining entrained particulate matter. The pressure in the quench tank is substantially the same as the gas generator located above. A portion of the quench water at the bottom of the quench tank is removed by way of a lockhopper system and settler, such as shown in coassigned U.S. Pat. No. 3,607,157. Another stream of quench water carrying fine particles exits the gasifier quench chamber in response to a liquid level controller and is directed to a settler. Clarifier bottoms or tops are separated from the water and have a composition similar to the previously described carbon-rich particulate matter. Alternatively, the hot raw effluent gas stream from the reaction zone may be partially cooled, by indirect heat exchange, prior to being scrubbed with water, by being passed through a radiant or convection gas cooler. For example, see coassigned U.S. Pat. Nos. 2,931,715; 4,081,253; and 4,377,132; which are incorporated herein by reference. Coarse slag particles and carbon-rich particulate material may pass from the water sump of the gas cooler and be collected in a lock hopper vessel. The solids and water from the lock hopper may then flow by gravity into a water sump or settler where optionally the coarse slag particles and the finer carbon-rich particulate material are removed and separated from each other. For example, a portion of the quench water at the bottom of the quench tank 26 is

removed by way of a lockhopper 37 and settler 40 as shown in the drawing for coassigned U.S. Pat. No. 3,544,291, which is incorporated herein by reference. The aqueous suspensions of particulate matter selected from the group consisting of coarse slag, carbon-rich particulate matter and mixtures thereof in lines 39, 41 and 42 of U.S. Pat. No. 3,544,291 have solids concentrations in the range of about 1.0 to 50.0 wt. %, such as about 10 to 20 wt. %. For example, the overflow stream in line 41 of the drawing in coassigned U.S. Pat. No. 3,544,291 may have a solids content of carbon-rich particulate matter in the range of about 1.0-4.0 wt. %. The underflow in line 42 may have a solids content of coarse slag particulate matter in the range of about 5 to 50 wt. %. Conventional solids-liquid separators e.g. screens may be used to recover the solid particles from the water. The coarse slag may be used as filler material. It was unexpectedly found that increased carbon conversion can be obtained when the carbon-rich particulate material either by itself or in admixture with a supplemental fuel is subjected to the partial oxidation process at a pressure which is less than that in the partial oxidation gasifier used to produce said carbon-rich particulate material starting with a bituminous coal.

A fuel mixture for the second partial oxidation reaction is prepared comprising about 20 to 100 wt. %, such as about 25 to 90 wt. %, of said carbon-rich particulate material and the remainder, if any, comprising a supplemental fuel selected from the group consisting of liquid hydrocarbonaceous fuel, coal, petroleum coke, and mixtures thereof. A mixture of said solid carbonaceous fuels, for example preferably bituminous coal in admixture with said carbon-rich particulate material may be introduced into a partial oxidation gas generator as an aqueous slurry having a solids content in the range of about 30-65 wt. %, or alternatively as crushed solid fuel mixture entrained in a gaseous medium selected from the group consisting of steam, recycle portion of the product gas,  $\text{CO}_2$ ,  $\text{N}_2$ , and mixtures thereof. The fuel mixture is introduced into a free-flow unobstructed noncatalytic vertical refractory-lined partial oxidation gas generator along with a free-oxygen containing gas and a temperature moderator by means of a burner, in the manner previously described. The  $\text{H}_2\text{O}$ /fuel wt. ratio is substantially in the same range as previously described in the first partial oxidation step. Advantageously, because of the high reactivity of the carbon-containing material, the O/C atomic ratio may be reduced in the second partial oxidation reaction for example, to a value in the range of about 0.6 to 1.3.

The second partial oxidation reaction takes place in a reducing atmosphere at an autogenous temperature in the range of about 2000° F. to 2700° F., and at a reduced pressure in the range of about 1 to 16 atmospheres and at least 16 atmospheres below the pressure in the first partial oxidation step in which the first carbon-rich particulate material was produced. A raw product gas stream comprising synthesis gas, reducing gas, or fuel gas having a composition substantially as previously described and containing entrained molten slag and less 60 carbon-containing particulate material than that produced when said fuel mixture is reacted by partial oxidation at substantially the same operating conditions as in the second partial oxidation reaction step except for a higher pressure, which pressure is in the same range as 65 that in the first partial oxidation reaction step. For example, from about 1.0 to 10.0 wt. % of carbon-rich particulate material (basis weight of carbon in bitumi-

nous coal) is produced during the first partial oxidation step with a feedstock of bituminous coal only. In contrast, from about 0.01 to 2.0 wt. % of carbon-rich particulate material (basis weight of carbon in all of the fuel fed to the second partial oxidation step) is produced during the second partial oxidation step with a fuel feed comprising carbon-rich particulate material produced in the first partial oxidation step with or without admixture with fresh supplemental fuel. Accordingly, by the subject process in the second partial oxidation step more carbon is converted into carbon oxides at a greater process efficiency. For example, less oxygen is consumed in the second partial oxidation step to convert the same amount of carbon as that converted in the first partial oxidation step into synthesis gas. Further, substantial cost savings are effected by the subject process since costs for oxygen and for cleaning the process gas stream are reduced.

The hot raw gas stream is cooled by quenching in water and/or by indirect heat exchange in a radiant and/or convection cooler. Slag is separated from the raw gas stream.

In another embodiment, an additive selected from the group consisting of iron-containing material, copper-containing material, calcium-containing material, a mixture of iron-containing material and calcium-containing material, and a mixture iron-containing material and silicon-containing material is introduced into the gas generator in the first partial oxidation step. Removal of sulfur-containing gases and/or molten slag, including vanadium laths and spinels as found in the bituminous coal, from the refractory lined reaction zone is thereby facilitated. For example, from about 1 to 10 parts by weight of additive, such as about 0.1 to 5 parts by weight of additive are used for each part by weight of ash in the bituminous coal. For example, see coassigned U.S. Pat. Nos. 4,668,428; 4,668,429; 4,657,698; 4,732,700; and 4,826,627, which are incorporated herein by reference.

During the first partial oxidation reaction most of the aforesaid additive e.g. greater than 80 wt. % goes into the coarse slag. The remainder of the additive goes into the carbon-rich particulate material and is therefore available to facilitate removal of sulfur-containing gases and/or molten slag in the second partial oxidation stage.

The process of the invention has been described generally and by examples with reference to materials of particular composition for purposes of clarity and illustration only. It will be apparent to those skilled in the art from the foregoing that various modifications of the process and materials disclosed herein can be made without departure from the spirit of the invention.

We claim:

1. A partial oxidation process for producing synthesis gas, reducing gas or fuel gas from bituminous coal comprising the steps of:

(1) reacting said bituminous coal by partial oxidation with a free-oxygen containing gas and a temperature moderator in a free-flow vertical refractory-lined gas generator at an autogenous temperature in the range of about 2000° F. to 2700° F., a pressure in the range of about 17 to 100 atmospheres, an O/C atomic ratio in the range of about 0.7 to 1.6, and a weight ratio of  $\text{H}_2\text{O}$  to bituminous coal in the range of about 0.10 to 5.0, to produce a raw gas stream comprising synthesis gas, reducing gas, or fuel gas with entrained molten slag and carbon-rich particulate material;

- (2) cooling said raw gas stream from (1) and separating therefrom coarse slag and carbon-rich particulate material;
- (3) reacting a fuel comprising from about 20 to 100 wt. % of said carbon-rich particulate material and any remainder comprising a supplemental fuel selected from the group consisting of liquid hydrocarbonaceous fuel, coal, petroleum coke, and mixtures thereof by partial oxidation with a free-oxygen containing gas and a temperature moderator in a free-flow vertical refractory-lined gas generator at an autogenous temperature in the range of about 2000° F. to 2700° F., a pressure in the range of about 1 to 16 atmospheres and at least 16 atmospheres below the pressure in the gas generator in (1), an O/C atomic ratio in the range of about 0.6 to 1.3, and a weight ratio of  $H_2O$  to fuel mixture in the range of about 0.1 to 5.0, to produce a raw product gas stream comprising synthesis gas, reducing gas, or fuel gas with entrained molten slag and containing less carbon-rich particulate material than that produced when said fuel mixture is reacted by partial oxidation at substantially the same operating conditions as those in the gas generator in (3) except for a higher pressure which is in the range of about 17 to 100 atmospheres; and
- (4) cooling said raw gas stream from (3).

2. The process of claim 1 wherein the bituminous coal in (1) is introduced into the gas generator as an aqueous slurry having a solids content in the range of about 30-65 wt. %, or alternatively as crushed bituminous coal entrained in a gaseous medium selected from the group consisting of steam, recycle portion of the product gas,  $CO_2$ ,  $N_2$ , and mixtures thereof.

3. The process of claim 2 wherein said bituminous coal has a particle size such that 100% passes through an ASTM E11-70 Sieve Designation Standard (SDS) 1.40 mm Alternative No. 14.

4. The process of claim 1 provided with the steps of quench cooling of the raw gas stream from (1) in a pool of quench water; whereby said molten slag solidifies into said coarse slag; separating said coarse slag and carbon-rich particulate matter in a settler or clarifier; and mixing together said carbon-rich particulate matter, settler and clarifier bottoms, and said supplemental fuel to provide said fuel mixture for reacting in (3).

5. The process of claim 1 provided with the steps of cooling the raw gas stream from (1) by passing it through a radiant and/or convection gas cooler followed by scrubbing the gas stream with water; whereby, said molten slag solidifies into said coarse slag; separating said coarse slag and carbon-rich particulate matter in a settler or clarifier; and mixing together said carbon-rich particulate matter, settler or clarifier bottoms, and said supplemental fuel to provide said fuel mixture for reacting in (3).

6. The process of claim 1 wherein the partial oxidation reactions in (1) and (3) take place in the same or different gas generators.

7. The process of claim 1 wherein about 1.0 to 10.0 wt. % of carbon-rich particulate material (basis weight of carbon in bituminous coal) is produced in (1) and about 0.01 to 2.0 wt. % of carbon-rich particulate mate-

rial (basis weight of carbon in fuel fed to gas generator in (3)) is produced in (3).

8. The process of claim 1 wherein the fuel mixture reacted in (3) is introduced into the gas generator as an aqueous slurry having a solids content in the range of about 30-65 wt. %, or alternatively as crushed fuel mixture entrained in a gaseous medium selected from the group consisting of steam, recycle portion of the product gas,  $CO_2$ ,  $N_2$ , and mixtures thereof.

9. The process of claim 1 provided with the step of introducing an additive into the gas generator in (1) to facilitate the removal of sulfur-containing gases and/or molten slag including vanadium-laths and spinels.

10. The process of claim 9 wherein from about 1 to 10 parts by weight of additive are introduced into the gas generator in (1) for each part by weight of ash in the bituminous coal.

11. The process of claim 9 wherein said additive is selected from the group consisting of iron-containing material, copper-containing material, calcium-containing material, a mixture of iron-containing material and calcium-containing material, and a mixture iron-containing material and silicon-containing material.

12. The process of claim 1 wherein the supplemental fuel in (3) is a solid carbonaceous fuel.

13. A partial oxidation process for producing synthesis gas, reducing gas or fuel gas from bituminous coal comprising the steps of:

(1) reacting said bituminous coal by partial oxidation with a free-oxygen containing gas and a temperature moderator in a free-flow vertical refractory-lined gas generator at an autogenous temperature in the range of about 2000° F. to 2700° F., a pressure in the range of about 17 to 100 atmospheres, an O/C atomic ratio in the range of about 0.7 to 1.6, a weight ratio of  $H_2O$  to carbon in the fuel mixture in the range of about 0.1 to 5.0, to produce a raw gas stream comprising synthesis gas, reducing gas, or fuel gas with entrained molten slag and carbon-rich particulate material;

(2) cooling said raw gas stream from (1) and separating therefrom coarse slag and carbon-rich particulate material;

(3) reacting a fuel mixture comprising from about 25 to 90 wt. % of said carbon-rich particulate material and the remainder comprising, bituminous coal by partial oxidation with a free-oxygen containing gas and a temperature moderator in a free-flow vertical refractory-lined gas generator at an autogenous temperature in the range of about 2000° F. to 2700° F., a pressure in the range of about 1 to 16 atmospheres and at least 16 atmospheres below the pressure in the gas generator in (1), an O/C atomic ratio in the range of about 0.6 to 1.3, and a weight ratio of  $H_2O$  to bituminous coal in the range of about 0.1 to 5.0, to produce a raw product gas stream comprising synthesis gas, reducing gas, or fuel gas with entrained molten slag and containing less carbon-rich particulate material than that produced when said fuel mixture is reacted by partial oxidation at substantially the same operating conditions as those in the gas generator in (3) except for a higher pressure which is in the range of about 17 to 100 atmospheres; and

(4) cooling said raw gas stream from (3).

\* \* \* \* \*